

# UNITED STATES PATENT OFFICE.

JOHN STUART CAMPBELL, OF LONDON, ENGLAND.

## VULCANIZABLE COMPOSITION OF MATTER HAVING COMMINUTED LEATHER AS A BASE AND METHOD OF PREPARING SAME.

1,302,463.

Specification of Letters Patent. Patented Apr. 29, 1919.

No Drawing.

Application filed September 17, 1917. Serial No. 191,750.

*To all whom it may concern:*

Be it known that I, JOHN STUART CAMPBELL, a subject of the King of Great Britain and Ireland, residing at Room 35, Broad 5 Street House, New Broad Street, London, E. C. 2, England, have invented a new and useful Vulcanizable Composition of Matter Having Comminuted Leather as a Base and Methods of Preparing Same, of which 10 the following is a specification.

This invention consists in a new and useful vulcanizable composition of matter and a method of preparing same, the said composition containing comminuted or disintegrated leather as a base and being suitable in its vulcanized state for most of the purposes for which leather, india rubber or the like are used, besides being capable of being reduced to a semi-fluid state before it is vulcanized so that it can be applied on a canvas or other backing and then vulcanized. The comminuted leather is preferably obtained by grinding or disintegrating waste or scrap leather.

25 Many compositions are known which contain comminuted or disintegrated leather as a base together with fibrous material, filling material, oils or fats, and rubber or some other binding agent, and as compared 30 with such compositions the characteristic feature of the present invention consists in that the comminuted or disintegrated leather is subjected to preliminary treatment for the purpose of eliminating entirely the 35 fatty matter naturally in the leather.

The essential ingredients of the new composition are disintegrated or comminuted leather which has been boiled in water containing sufficient caustic alkali to saponify 40 the fatty matter in the leather, and a vulcanizable gum such as rubber, caoutchouc, balata or like resilient and vulcanizable binding material. Any desired filling material and any required coloring and preserving 45 agents may be added. The vulcanizing agent may be introduced at any stage. The preferred filling materials are magnesia or asbestos fiber or asbestos dust (about 15% of the weight of the comminuted 50 leather if a product resembling leather be required) fibrous material such as hair or wool or animal or vegetable fiber, chalk or whitening, (about 5%) and lime, (about 2%). The proportions of the resilient vulcanizable binding material will vary with 55

the degree of elasticity required in the finished product—about 15% of the weight of the comminuted leather yielding a product resembling leather.

The preferred method of preparing the 60 said composition consists firstly in boiling the leather, after it has been ground to powder, in water containing sufficient caustic alkali to saponify the fatty matter naturally in the leather, until the leather has been 65 converted into a jelly-like mass—which will usually occur in about an hour and a half. The filling material and, if desired, the sulfur or other vulcanizing agent and any required coloring and preserving agents, may 70 then be added and thoroughly mixed with the jelly-like mass, in which case the boiling is continued until the ingredients are thoroughly incorporated with each other. It is not essential however to make these 75 additions at this stage; they may be made during the subsequent mixing stage. In either case, the mass after boiling is dried, for example in vacuum pans or trays, until it crumbles readily to powder. 80

In the mixing stage, the elastic gum or rubber or like resilient and vulcanizable binding material is introduced between heated mixing rollers and the dried mass obtained as hereinbefore described is incorporated with it. If the filling material and other ingredients have not been added during the boiling stage they are now added together with the sulfur or other vulcanizing 85 agent. 90

The product is then calendered into sheets of the desired thickness or molded into the desired shape or form and vulcanized; or, if sheets or bands capable of withstanding considerable tension are required, the said 95 product is rendered more or less fluid by means of a suitable solvent and applied upon a backing, such as canvas, and afterward vulcanized.

During the mixing and rolling operation, 100 steel or metal dust may be added for the purpose of rendering the resultant product particularly suitable for hard wear.

Among the many uses of the composition may be mentioned the production of solid 105 tires, washers, hydraulic rings, valves, the soles of boots, and molded articles. Sheets of the material may be embossed or ornamented by passing them between suitably engraved rolls.

When the composition is to be applied upon a canvas or like backing for the purpose of making belts, tire-covers, linings, waterproof sheets or the like it may be rendered semi-fluid by means of a solvent such as naphtha.

By suitably regulating the proportions of the ingredients and the degree of vulcanization a material suitable for electrical insulation is produced. The hardness of the material may be varied to suit requirements, and is largely dependent upon the amount of the sulfur or other vulcanizing agent and the temperature and time of vulcanization.

What I claim as my invention and desire to secure by Letters Patent is:—

1. A vulcanizable composition having comminuted or disintegrated leather as a base, the essential constituents of which are comminuted or disintegrated leather which has been boiled in water containing sufficient caustic alkali to saponify the fatty matter in the leather, but not sufficient to dissolve the leather, and a resilient vulcanizable binding material, the said constituents being thoroughly mixed and incorporated with each other, under the action of heat to form a homogeneous mass.

2. A vulcanizable composition consisting of comminuted or disintegrated leather which has been boiled in water containing

sufficient caustic alkali to saponify the fatty matter in the leather, but not sufficient to dissolve the leather, magnesia, whitening, lime and a resilient vulcanizable binding material, 35 incorporated with each other and with vulcanizing, coloring and preserving agents, under the action of heat to form a homogeneous mass substantially as set forth.

3. A method of preparing the composition 40 claimed in claim 1, consisting in grinding scrap leather to powder and boiling same in water containing sufficient caustic alkali to saponify the fatty matter in the leather, but not sufficient to dissolve the leather, then 45 drying and thoroughly mixing and incorporating the powder thus treated with a resilient vulcanizable binding material, under the action of heated mixing rollers.

4. The mode herein described of improv- 50 ing the quality of vulcanizable compounds of comminuted leather and rubber, the said mode consisting in boiling the comminuted leather in water containing sufficient caustic alkali to saponify the fatty matter in 55 the leather, but not sufficient to dissolve the leather and then incorporating same with the rubber.

In testimony whereof I have signed my name to this specification.

JOHN STUART CAMPBELL.